# EUROPEAN PATENT SPECIFICATION

(11) **EP 0 106 686 B1**
(45) Date of publication and mention of the grant of the patent: **20.12.1989**
(21) Application number: 83306250.8
(22) Date of filing: 14.10.1983
(51) Int. Cl.: D02G 1/02

(54) **Intermittently textured yarn**
Abwechselnd texturiertes Garn
Fil texturé par intermittence

(30) Priority: 18.10.1982 US 434898; 18.10.1982 US 434899; 18.10.1982 US 434900; 18.10.1982 US 434909; 18.10.1982 US 435052; 18.10.1982 US 435053; 10.11.1982 US 440497; 10.11.1982 US 440498; 22.02.1983 US 468469
(43) Date of publication of application: 25.04.1984
(73) Proprietor: MILLIKEN RESEARCH CORPORATION, Spartanburg South Carolina 29304 (US)
(72) Inventor: Moore, James Ronald, Inman South Carolina 29349 (US); Pittman, Edgar Henry, Spartanburg South Carolina 19302 (US); Schroder, William John, Spartanburg South Carolina 29303 (US); Warner, Charles Erwin, Spartanburg South Carolina 29303 (US)
(74) Representative: Bass, John Henton

(56) References cited:
- GB-A- 1 362 178
- US-A- 3 100 091
- US-A- 3 350 867
- US-A- 3 797 775
- US-A- 3 911 655
- US-A- 4 033 103
- US-A- 4 345 424

## Description

This invention relates to a method and apparatus for producing a false twisted, continuous multifilament yarn, in which yarn is supplied from a supply package through a heater to a false twisting device.

A method and apparatus of this type is described in US-A-4 033 103, in which the thread bundle is intermittently or periodically deflected from its normally linear path and shortly before its entry into the false twister by means of a false twist blocking element placed in running contact with the thread bundle.

It is an object of the invention to provide an improved yarn processing system of the above type, and this is achieved by randomly varying the tension of the yarn being processed.

The particular quality of the random variation of tension which characterises this invention can conveniently be defined in two alternative but parallel ways.

On the one hand, the method of this invention may be characterised by intermittently and randomly varying the supply of yarn to the false twisting device, and driving the false twist device at a speed to produce a twist multiple between 250 and 450 in the multifilament yarn.

The term "twist multiple" (TM) is standard in the industry and is defined as where TPI is the number of turns per inch (25.4 mm) of twist imparted to the yarn and YD is the yarn denier (g/9000 m=0.1111 tex).

On the other hand, the method may be characterised by intermittently and randomly varying the tension of the yarn in the heater between a high range of 0.21 to 0.60 grams per denier and a low range of 0.06 to 0.21 grams per denier.

The apparatus of this invention is characterised by a disc type tension device located between said heater and said yarn supply to intermittently and randomly vary the flow of yarn from said supply to said false twist device, said false twist device being adapted to be driven at a speed to produce a twist multiple of between 250 and 450 in the multifilament yarn.

The invention is further described, by way of example only, with reference to the accompanying drawings in which:
Figure 1 is an overall schematic representation of the new and novel system to produce a textured, continuous filament synthetic yarn;
. Figure 2 is a partial perspective view of the yarn-supply creel for the system shown in Figure 1;
Figure 3 is an exploded schematic view of the yarn tension disc device used in the system of Figure 1;
Figure 4 is a top view of the post of the yarn tension disc device of Figure 3;
Figure 5 is a side elevation view of the post shown in Figure 4;
Figure 6 is a schematic representation of the voltage control scheme for the yarn tension disc electromagnet;
Figure 7 is a circuit diagram for the electromagnet of the yarn tension disc device;
Figure 4 is a graphical representation of the voltage supplied to the electromagnet of the yarn tension disc device; and
Figures 9 and 10 represent a modification of. the invention as shown in Figures 7 and 8, respectively.

Looking now to Figure 1, the overall system of Figure 1 will be explained to obtain the novel disclosed yarn. The system is directed to a method to produce a specially textured yarn by intermittently varying the draw of a continuous filament partially oriented, synthetic, multifilament yarn such as polyester. The multifilament yarn 10 is supplied from a supply package 12 to the false twist device 14 by the feed roll device 16. The yarn 10 from the package 12 successively, in its travel to the feed roll device 16, passes through the balloon control apparatus 18, over the guide members 20, 22 and 24 through the electro-magnetically controlled tension disc apparatus 26 and under the guide member 28 through the primary heater 30 and false twist device 14 to the feed roll device 16. The yarn 10 is intermittently and randomly drawn in the primary heater 30 by the intermittent hold back action of the disc tension apparatus 26. The discs 32 and 34 are intermittently and randomly drawn together and released on the yarn 10 by the action of the electromagnet 36 controlled by the varying voltage supplied thereto by a suitable voltage source which is varied by the action of a random signal generator.

From the feed roll device 16 the textured yarn passes through the secondary heater 37 with very little overfeed since the speed of the feed roll device 38 is substantially the same as the feed roll device 16 and the crimp in the yarn is allowed to set. Depending on the amount of crimp contraction desired the secondary heater can be turned on at an appropriate temperature or off or by-passed and the overfeed varied from high to very little.

The feed roll device 38 is driven at a higher speed than the feed roll device 44 to overfeed the textured yarn through the air jet entangling device 40 to commingle and entangle the individual filaments of the textured yarn. From the feed roll device 38 the entangled, textured yarn is slightly overfed to the yarn take-up package 42 by the feed roll device 44.

Schematically in Figure 1, the yarn package 12 and the balloon control element 18 are shown as separate items but in actual practice a creel unit, designated 46 in Figure 2, is used. The creel unit 46 supports a plurality of packages 12 for a plurality of false twist spindle positions and is slid in and out of position relative to a multiple spindle false twisting machine. In Figure 2 a partial creel is shown supporting a pair of supply packages held on creel pins supported by creel pin support members 48 that are connected to the creel. Also connected to the creel is a horizontal separation plate 50 through which the yarn guide supports 52 project. A yarn guide 54 for each yarn package is connected thereto to guide the yarn 10 from the package 12 towards the guide member 20. Mounted on both sides of the horizontal separator plate 50 is a channel beam 56 between which is connected the balloon control apparatus or bar 18. The balloon of yarn from the creel is unusually erratic and violent due to the alternating take-off velocity and is therefore prone to entanglement if not controlled. As shown in Figure 2 the bar 18 prevents yarn 10 from the package 12 from forming a full balloon and getting entangled in and around various elements of the creel such as yarn guides 54. As shown in Figure 2, a second bar 18 is shown which is used for the same purpose for the yarn packages (not shown) on the opposite side of the creel unit 46.

Figures 3-5 show the electromagnetically controlled tension disc apparatus 26 in detail. The apparatus 26 basically consists of the electromagnet 36, the spring biasing member 60 of Teflon or other suitable material, the tension discs 32 and 34, the disc post 62 and the screw 63 to maintain the aforementioned element in operative relationship. The disc 32 is made from a magnetically attractable material such as a ferrous material while the disc 34 is manufactured from a non-magnetically attractable material. For reasons hereafter explained the post 62 has a slot 64 therein which is off set from the centerline of the post. Also for reasons hereinafter explained, it is desired to supply random, intermittent pulses of low and high D.C. voltage with a superimposed A.C. voltage to cause the discs 32 and 34 to close randomly and intermittently and to cause the discs to vibrate relative to one another and relative to the electromagnet 36. To accomplish this action the arrangement shown in Figure 6 and the circuit shown in Figure 7 are employed. Basically, the voltage to the electromagnet 36 is supplied from a control box 65 which receives voltage from an A.C. power supply 66, a high voltage D.C. power supply 68 and a low voltage D.C. power supply 70. Connected between the high voltage D.C. source 68 and the control box 65 is a random signal generator 72 of the type disclosed in U.S. Patent Number 4,160,359 which intermittently and randomly interrupts the voltage from the high voltage D.C. source to the control box 65. Located in each circuit to the electromagnet 36 is a diode 74 which only allows current to flow in one direction towards the electromagnet 36. Schematically represented in the high and low voltage D.C. circuit is an adjust switch or variable resistor 76 to adjust the D.C. voltage in the respective circuit.

As represented in the graph of Figure 8, the A.C. voltage from the source 66 supplies A.C. voltage continuously while the high D.C. voltage from the source 68 is interrupted randomly and continuously by the random signal generator 72. As indicated in the graph, this provides periods of high voltage 78 and low voltage 80 for different durations of time, as well as peaks 82 at times when the high voltage D.C. current is not being supplied and the A.C. current is at its positive peak on its cycle. The various lengths of the high voltage peak 78 represent periods when the yarn 10 is being held tightly between the discs 32 and 34 while the peaks 82 and the low voltage periods 80 represent periods when the voltage is low and the discs 32 and 34 tend to release the grip on the yarn 10 and vibrate as the yarn passes therethrough. At these times the spring biasing member 60 causes the discs to be urged upward and allows the frictional resistance between the discs 32 and 34 and between the disc 34 and the electromagnet 36 to be reduced so that the torque exerted by the yarn passing through the slot 64 of the post 62 will cause them to rotate more efficiently to provide the self-cleaning action. The vibration of the discs allows the discs to be rotated more easily so that the yarn passing through will subsequently clean out the finish deposited between the discs by the yarn.

Looking now to Figures 9 and 10 an alternate scheme is shown to enhance the rotation of the discs 32 and 34. In Figures 9 and 10, elements therein which are the same in Figures 1-8 are indicated by the same reference number. The basic modification shown in Figures 9 and 10 is the inclusion of a timer 100 in the low voltage D.C. circuit to momentarily cut-off the current flow in the D.C. circuit to the electromagnet 36 to allow the A.C. voltage to peak as indicated in Figure 10. It is understood that the current in the A.C. circuit is flowing continuously in order to obtain the result shown in Figure 10. During periods when the timer 100 has the low voltage D.C. circuit open and the random signal generator 72 has the high voltage D.C. circuit open, only half-wave rectified A.C. voltage is applied to the coil as shown in Figure 10. This will momentarily upset the tension of the yarn, but enhances the rotation of the discs 32 and 34.

Alternatively, the wall 84 defining one portion of the slot 64 can be eliminated and replaced by an upstanding guide member, not shown, which will serve to confine the yarn path to a path offset from the centerline of the post 62.

In the preferred form of the invention the spring biasing member 60 is of a diameter greater than the inner, internal diameter 85 and less than the inner, external diameter 86 of the lower tension disc 34 so that it is curved downward at its extremities when the discs 32 and 34 are pulled towards the electromagnet 36. Conversely, when the voltage to the electromagnet is reduced, the upward force exerted due to the bias of the member 60 urges the discs upward.

As described briefly before, it is desired to cause the tension discs 32 and 34 to rotate in order to dissipate the finish deposited therebetween by the yarn 10. As described above, the discs 32 and 34 are free to rotate on the post 62. To further enhance this rotation, the slot 64 is located off center of the centerline of the post so that the yarn passing between the discs 32 and 34 will exert a torque thereon. Furthermore, since yarn 10 is located in the slot 64 between the discs 32 and 34, the yarn cannot jump out from between the discs and have to be rethreaded. Further, such location of the yarn in the slot prevents uncontrolled texturing and lessens the tendency for yarn breaks.

In the form described hereinabove the preparation of a single end of multifilament synthetic yarn is described but, depending on the ultimate use of the yarn produced, a plurality of yarns can be interlaced or commingled in the air jet 40. Examples of such yarn are set forth below.

### Example 1

Two ends of a 240 denier (27 tex), 68 filament DuPont 56T polyester yarn were processed as described above and entangled or interlaced in the air jet 40 to provide a 2/150/68 yarn with an actual denier of 321 (35.6 tex). The elongation was 51% with a crimp contraction of 1%. The operating conditions were as follows:

The yarn thus produced has a very low crimp contraction with high luster and intermittent character.

### Example 2

Two ends of a 220 denier (24 tex), 54 filament DuPont 693T polyester yarn were processed and entangled in the air jet 40 to provide a 2/150/54 yarn with an actual diameter of 328 denier (36.4 tex). The elongation was 48% with a crimp contraction of 1.8%. The operating conditions were as follows:

The yarn produced has a low crimp contraction with very high luster and intermittent character.

It can readily be seen that the described apparatus and method provides a randomly, intermittently textured, continuous multifilament synthetic yarn which along its length has variable molecular orientation, bulk, torque, twist and shrinkage. The produced yarn has a low crimp contraction and a high luster. This yarn is especially useful in the fabrication of a velvet-type upholstery fabric and provides unique visual effects due to its variable dye affinity.

## Claims

1. Method to produce a false twisted, continuous multifilament synthetic yarn comprising the steps of: supplying a continuous multifilament yarn from a supply package through a heater to a false twisting device and allowing the yarn to be set after false twisting and taking up the false twisted yarn, characterised by intermittently and randomly varying the supply of yarn to the false twisting device, and driving the false twist device at a speed to produce a twist multiple between 250 and 450 in the multifilament yarn.

2. The method of claim 1 wherein the false twisted yarn is entangled in an air entanglement device prior to take-up.

3. Method to produce a false twisted, multifilament synthetic yarn comprising the steps of: supplying a continuous multifilament yarn from a supply package through a heater to a false twisting device, driving the false twist device at a speed to produce a false twist in the multifilament yarn, allowing the yarn to set after false twisting and taking up the false twisted yarn, characterised by intermittently and randomly varying the tension of the yarn in the heater between a high range of 0.21 to 0.60 grams per denier and a low range of 0.06 to 0.21 grams per denier.

4. Apparatus to produce a false twisted multifilament yarn by the method of claim 1 or 3, comprising: a yarn supply (12), a false twist device (14), a heater (30) located between said yarn supply and said false twist device and take-up means (42) to take-up the false twisted yarn, characterised by disc type tension device. (26) located between said heater and said yarn supply to intermittently and randomly vary the flow of yarn from said supply to said false twist device, said false twist device being adapted to be driven at a speed to produce a twist multiple of between 250 and 450 in the multifilament yarn.

5. The apparatus of claim 4 wherein an air jet commingling device (40) is located between said false twist device (14) and to takeup means (42).

6. The apparatus of claims 4 or 5 wherein a bar member (18) is mounted between said yarn supply (12) and said false twist device (14) to prevent the yarn from forming a full balloon path.

7. The apparatus of claims 4 or 5 wherein said disc type tension device (26) includes an electromagnet (36), a post member (62) operably associated with said electromagnet, a first metallic disc member (32) mounted on said post, a second metallic disc member (34) mounted on said post adjacent said first disc member, a D.C. circuit (68, 70) supplying said electromagnet and an A.C. supply (66) to said electromagnet operable to periodically allow said first and second disc members to move relative to one another and relative to the electromagnet.

8. The apparatus of claim 7 wherein said D.C. circuit includes a high voltage source (68) and a low voltage source (70) and means (72) to periodically interrupt the high voltage source.

9. The apparatus of claim 8 wherein said A.C. voltage is intermediate of the high and low D.C. voltage.

10. The apparatus of claims 7, 8 or 9 wherein said post member (62) has a slot (64) therein offset from the centerline of said post.

11. The apparatus of claims 7, 8, 9, or 10, wherein a spring biasing member (60) is mounted on said post (62) between said electromagnet (36) and said discs (32, 34) to exert an upward force on said discs. 12. The apparatus of claim 11 wherein said discs (32, 34) are dish shaped with the bottom disc curving downward, said spring biasing means (60) conforming to the internal shape of said bottom disc (34) and having a diameter less than internal outer diameter of said bottom disc but greater than the internal inner diameter of said bottom disc whereby said spring biasing means is curved downward by said bottom disc when voltage is applied to said electromagnet.

13. The apparatus of any of claims 7 to 12 wherein the A.C. is supplied continuously and said D.C. circuit includes a means (72) to momentarily interrupt the flow of direct current to said electromagnet.

## Patentansprüche

1. Verfahren zum Herstellen eines mit Falschdraht gezwirnten endlosen synthetischen Multifil-Garns, mit den folgenden Schritten: Liefern eines endlosen Multifil-Garns von einer Lieferspule über eine Heizvorrichtung an eine Falschdraht - Zwirnvorrichtung und Fixierenlassen des Garns nach dem Falschdrahtzwirnen und Aufwickeln des mit Falschdraht gezwirnten Garns, gekennzeichnet durch intermittierendes und zufälliges Variieren der Garnlieferung an die Falschdraht - Zwirnvorrichtung, und Betreiben der Falschdraht - Zwirnvorrichtung mit einer Geschwindigkeit, bei der eine Drehungszahl zwischen 250 und 450 im Multifil-Garn entsteht.

2. Verfahren nach Anspruch 1, bei dem das mit Falschdraht gezwirnte Garn vor dem Aufwickeln in einer Luftstrom-Verschlingvorrichtung verwirrt wird.

3. Verfahren zum Herstellen eines mit Falschdraht gezwirnten synthetischen Multifil-Garns, mit den Schritten: Liefern eines endlosen Multifil-Garns von einer Lieferspule über eine Heizvorrichtung an eine Falschdraht - Zwirnvorrichtung, Betreiben der Falschdraht - Zwirnvorrichtung mit einer Geschwindigkeit, bei der im Multifil-Garn ein Falschdraht entsteht, Fixierenlassen des Garns nach dem Falschdrahtzwirnen und Aufwickeln des mit Falschdraht gezwirnten Garns, gekennzeichnet durch intermittierendes und zufälliges Variieren der Garnzugspannung in der Heizvorrichtung zwischen einem hohen Bereich von 0,21 bis 0,60 Gramm je Denier und einem unteren Bereich von 0,06 bis 0,21 Gramm je Denier.

4. Vorrichtung zum Herstellen eines mit Falschdraht gezwirnten Multifil-Garns nach dem Verfahren gemäß Anspruch 1 oder 3, mit einem Garnvorrat (12), einer Falschdraht - Zwirnvorrichtung (14), einer zwischen dem Garnvorrat und der Falschdraht - Zwirnvorrichtung angeordneten Heizvorrichtung (30) und einer Vorrichtung (42) zum Aufwickeln des mit Falschdraht gezwirnten Garns, gekennzeichnet durch eine zwischen der Heizvorrichtung und dem Garnvorrat angeordnete Scheiben - Belastungsvorrichtung (26), welche den Garnlauf vom Vorrat zur Falschdraht - Zwirnvorrichtung intermittierend und zufällig zu variieren vermag, wobei die Flaschdraht - Zwirnvorrichtung mit einer Geschwindigkeit betreibbar ist, bei der eine Drehungszahl von zwischen 250 und 450 im Multifil-Garn entsteht.

5. Vorrichtung nach Anspruch 4, bei der zwischen der Falschdraht - Zwirnvorrichtung (14) und der Aufwickelvorrichtung (42) eine Luftstrom - Verschlingvorrichtung (40) angeordnet ist.

6. Vorrichtung nach Anspruch 4 oder 5, bei der zwischen dem Garnvorrat (12) und der Falschdraht - Zwirnvorrichtung (14) eine Stange (18) angeordnet ist, welche die Vollausbildung eines Bauchs im Garniauf verhindert.

7. Vorrichtung nach Anspruch 4 oder 5, bei der die Scheiben - Belastungsvorrichtung (26) einen Elektromagneten (36), eine mit dem Elektromagneten betreibsmäßig verbundene Achse (62), eine auf der Achse angeordnete erste metallische Scheibe (32), eine auf der Achse nahe der ersten Scheibe angeordnete zweite metallische Scheibe (34), eine Gleichspannungs - Schaltungsanordnung (68, 70) zur Versorgung des Elektromagneten und eine Wechselspannungs - Quelle (66) zum Elektromagneten umfaßt, welche so betreibbar ist, daß sie periodisch eine Bewegung der ersten und der zweiten Scheibe relativ zueinander und relativ zum Elektromagneten ermöglicht.

8. Vorrichtung nach Anspruch 7, bei der die Gleichspannungs - Schaltungsanordnung eine Hochspannungs - Quelle (68) und eine Niederspannungs - Quelle (70) und Mittel (72) zum periodischen Unterbrechen der Hochspannungs - Quelle umfaßt.

9. Vorrichtung nach Anspruch 8, bei der die Wechselspannung zwischen der hohen und der niedrigen Gleichspannung liegt.

10. Vorrichtung nach Anspruch 7, 8 oder 9, bei der in der Achse (62) ein gegenüber der Achsenmittellinie versetzter Schlitz (64) ausgebildet ist.

11. Vorrichtung nach Anspruch 7, 8, 9 oder 10, bei der auf der Achse (62) zwischen dem Elektromagneten (36) und den Scheiben (32, 34) ein federndes Vorspannorgan (60) angeordnet ist, das auf die Scheiben eine aufwärts gerichtete Kraft ausübt.

12. Vorrichtung nach Anspruch 11, bei der die Scheiben (32, 34) tellerförmig sind, wobei die untere Scheibe nach unten gekrümmt ist, das federnde Vorspannorgan (60) an die Innenform der unteren Scheibe (34) angepaßt ist und von kleinerem Durchmesser als der innere Außendurchmesser, aber von größerem Durchmesser als der innere Innendurchmesser der unteren Scheibe ist, derart, daß das federnde Vorspannorgan von der unteren Scheibe nach unten gekrümmt wird, wenn am Elektromagneten Spannung anliegt.

13. Vorrichtung nach einem der Ansprüch 7 bis 12, bei der die Wechselspannung ständig anliegt und die Gleichspannungs - Schaltungsanordnung eine Einrichtung (72) zur kurzzeitigen Unterbrechung des Gleichstromflusses zum Elektromagneten umfaßt.

## Revendications

1. Procédé de production d'un fil synthétique multifilament continu à fausse torsion, comportant des étapes dans lesquelles: on fournit à un dispositif de fausse torsion, via un dispositif chauffant, un fil multifilament continu provenant d'un enroulement d'alimentation et on permet au ful de se stabiliser après la fausse torsion puis on enroule le fil muni d'une fausse torsion, caractérisé en ce que l'on modifie aléatoirment et par intermittence la fourniture de fil au dispositif de fausse torsion et l'on entraîne le dispositif de fausse torsion à une vitesse produisant un coefficient de torsion entre 250 et 450 dans le fil multifilament.

2. Procédé selon revendication 1, dans lequel le fil doté d'une fausse torsion est emmmêlé dans un dispositif d'emmmêlement par air avant d'être enroulé.

3. Procédé pour produire un fil synthétique multifilament doté d'une fausse torsion, comprenant des étapes dans lesquelles: on fournit à un dispositif de fausse torsion, via un dispositif chauffant, un fil multifilament continu provenant d'un enroulement d'alimentation, on entraîne le dispositif de fausse torsion à une vitesse apte à produire une fausse torsion dans le fil multifilament, on permet au fil de se stabiliser après la fausse torsion et l'on enroule le fil doté de fausse torsion, caractérisé par le fait que l'on modifie de manière intermittente et aléatoire la tension du fil dans le dispositif chauffant, entre une plage haute de 0,21 à 0,60 grammes par denier et une plage basse de 0,06 à 0,21 grammes par denier.

4. Dispositif pour produire un fil multifilament doté de fausse torsion, par le procédé selon revendication 1 ou 3, comprenant: un distributeur de fil (12), un dispositif de fausse torsion (14), un dispositif chauffant (30) situé entre ladite alimentation de fil et ledit dispositif de fausse torsion, et des moyens d'enroulement (42) pour enrouler le fil doté de fausse torsion, caractérisé par un dispositif de tension du type à disques (26) situé entre ledit dispositif chauffant et ladite alimentation de fil, pour modifier aléatoirement et par intermittence le débit de fil provenant de ladite alimentation, fourni audit dispositif de fausse torsion, ledit dispositif de fausse torsion étant apte à être entraîné à une vitesse produisant un coefficient de torsion entre 250 et 450 dans le fil multifilament.

5. Dispositif selon la revendication 4, dans lequel un dispositif de combinaison à jet d'air (40) est disposé entre ledit dispositif de fausse torsion (14) et des moyens d'enroulement (42).

6. Dispositif selon revendications 4 ou 5, dans lequel un élément barre (18) est monté entre ladite alimentation de fil (12) et ledit dispositif de fausse torsion (14), pour empêcher le fil de former un trajet de ballon complet.

7. Dispositif selon revendications 4 ou 5, dans lequel ledit dispositif de tension du type à disques (26) comporte un électroaimant (36), un élément colonne (62) fonctionnellement associé audit électroaimant, un premier élément disque métallique (32) monté sur ladite colonne, un deuxième élément disque métallique (34) monté sur ladite colonne, en condition d'adjacence avec ledit premier élément disque, un circuit à courant continu (68, 70) alimentant ledit électroaimant et une alimentation de courant alternatif (66) pour ledit électroaimant, apte à opérer pour permettre périodiquement auxdits premier et deuxième élément disque de se mouvoir l'un par rapport à l'autre et par rapport à l'électroaimant.

8. Dispositif selon revendication 7, dans lequel ledit circuit de courant continu comprend une source de haute tension (68) et une source de basse tension (70) et des moyens (72) pour interrômpre périodiquement la source de haute tension.

9. Dispositif selon revendication 8 dans lequel ladite tension alternative est comprise entre la haute et la basse tension continue.

10. Dispositif selon revendications 7, 8 ou 9, dans lequel ledit élément colonne (62) est doté d'une fente (64) décalée par rapport à la ligne de centre de ladite colonne.

11. Dispositif selon revendications 7, 8, 9 ou 10, dans lequel un élément de sollicitation élastique (60) est monté sur ladite colonne (62) entre ledit électroaimant (36) et lesdits disques (32, 34), pour exercer une force ascendante sur lesdits disques.

12. Dispositif selon revendication 11, dans lequel lesdits disques (32, 34) sont en forme de cuvette, le disque inférieur étant courbé vers le bas, lesdits moyens de sollicatation élastique (60) se conformant à la forme interne dudit disque inférieur (34) et ayant un diamètre inférieure au diamètre extérieur interne dudit disque inférieure mais supérieur au diamètre intérieur interne dudit disque inférieur, par l'effet de quoi lesdits moyens de sollication élastique sont courbés vers le bas par ledit disque inférieur lorsque de la tension est appliquée audit électroaimant.

13. Dispositif selon l'une quelconque des revendications 7 à 12, dans lequel le courant alternatif est fourni de manière continue et ledit circuit de courant continu comporte des moyens (72) pour interrompre momentanément le passage du courant continu allant audit électroaimant.
